

July 20, 1937.

J. JOHNSTON

2,087,346

METHOD OF PRODUCING STEEL RAILS

Filed Aug. 21, 1930

*Fig. 1.*



*Fig. 2.*



INVENTOR

JOHN JOHNSTON.

BY

Usina & Pauber

ATTORNEYS

## UNITED STATES PATENT OFFICE

2,087,346

## METHOD OF PRODUCING STEEL RAILS

John Johnston, Short Hills, N. J., assignor to  
 United States Steel Corporation, New York,  
 N. Y., a corporation of New Jersey

Application August 21, 1930, Serial No. 476,868

9 Claims. (Cl. 148—21.5)

My invention relates to methods of making rails of steel or ferrous metal and more particularly to methods of controlling the cooling of rails after they have been rolled.

5 An object of the invention is to provide a method of controlling the cooling of rails such that the residual lengthwise tensile stresses which may occur in the head of finished rails are effectively reduced.

10 In making rails heretofore the rails, after having been rolled from a hot ingot, are permitted to cool by exposure to the atmosphere or to currents of air. This cooling is of sufficient rapidity to obviate undue softening of the metal and to 15 keep the area or space required by the rails while cooling within a commercially practicable and economic limit. The heat is given up by the rail to the atmosphere, or to the cooling air currents, from the exposed surface of the rail, and immediately heat from the interior of the rail begins to pass towards the somewhat cooler surface. This passage of heat necessarily involves a drop, or gradient, in temperature from the interior towards the surface of the rail, and 25 this gradient is greater the greater the rate of cooling and the consequent more rapid transfer of heat outwards through the cross section of the rail.

20 The temperature difference between the interior and the surface is also greater, the greater the cross-sectional dimension of the rail and the necessarily longer path of shortest travel of the heat. The temperature of the thinner parts of the rail, such as the web and flanges, in which 25 the ratio of extent of surface to volume is greater, also falls more rapidly than in the thicker parts, such as the head, in which the ratio of surface to volume is less. These differences are also greater the larger the rail. Under the relatively 30 rapid cooling now usual in practice, the temperature difference between the inner portion of the head and the web or flange may be quite appreciable, particularly in the larger and heavier rails.

35 Within a temperature range, notably from about 750° C. (1400° F.) to about 550° C. (1000° F.) steel undergoes transformations which are accompanied by a sharp increase in its volume. The exact temperature of initiation of these 40 transformations and the rate at which they proceed towards completion, depend primarily upon the composition of the steel, but also to some extent upon other factors such as the mode and rate of cooling. Because of the temperature differences through the rail section, alluded to

above, the completion of these transformations occurs at different times in different portions of the rail, being in general latest in those portions furthest away from the surface. The change in volume accompanying these transformations, 5 therefore, also occurs at different times in different portions of the rail; and consequently a series of stresses is set up in the rail in this period of its cooling.

These stresses may, with inappropriately rapid 10 cooling, be so considerable as to be potentially dangerous as internal sources of weakness, particularly in the temperature range before the fullest strength of the steel has developed; in any case they set up, in the finished cold rail, 15 a series of residual stresses which can, by appropriate means, be observed directly.

Systematic, direct, extended measurement of these residual stresses has shown that there may be, in the head of the rail, residual longitudinal 20 stress differences in excess of 10,000 pounds per square inch, some of these stresses being tensile, others compressive. It has also shown that the distribution of these residual stresses in the head of the rail depends upon the mode of cooling, 25 especially the rate of cooling through the temperature range in which the crystal transformations are proceeding; and that this distribution may, therefore, be controlled by appropriate control of the mode of cooling. These observations, 30 coupled with similar observations which show how these residual stresses in the head of the rail change when the rail is put in actual service, have led me to the belief that the head of a new rail should preferably be as free as practicable 35 from longitudinal tensile stresses, and that the stress gradient should preferably be uniform and not localized. It is the object of my invention to achieve this general result, and positively to 40 get rid of excessive stresses which are occasionally observed, particularly when the rail, in the earlier stages of its cooling, has for any reason been cooled too rapidly.

Further objects of my invention are to provide a method of controlling the cooling such that the 45 temperature differences in the cooling rail as it undergoes transformation, are minimized in a practical sense, and all parts of the rail transforms at substantially the same time and the same temperature.

With these and other objects in view, which will be apparent in the following description, the invention comprises the methods described in the following specification:

The various features of the apparatus are illus- 55

trated in the accompanying drawing, in which—  
Fig. 1 is a longitudinal vertical section, and

Fig. 2 is a transverse vertical section of an apparatus embodying a preferred form of my invention.

In my invention, the rails, as delivered from the rolls, are transferred to a hot-bed and permitted to cool at the usual or any desired rate until the rail is about approximately to the temperature of transformation for the particular steel comprising the rail. The particular temperature of transformation will vary with any given steel with respect to the rate of cooling from temperatures above the upper critical temperature. The rate of heat loss is then restricted, thus more nearly equalizing the temperature throughout the rail. The proper rate of loss of heat varies with the dimensions of the rails to be cooled, and must be adjusted accordingly. In all cases it should be sufficiently slow to enable all parts of the cross section of the rail to be within the temperature range of this transformation at approximately the same time and to enable the various parts of the rail, particularly in the head of the rail, to undergo the volume and structure change with a minimum of strain and distortion.

The cooling of the rail is continued at this retarded rate for a time after it has fallen below the transformation temperature, for example, it may be cooled at this rate to 550° C. (1000° F.) or even lower, thus ensuring the substantial completion of the structure and volume changes, and the maximum practicable equalization of such stresses as may have arisen, before the more rapid cooling to atmospheric temperature is resumed. Thereupon the normal, rapid or even an enhanced rate of cooling may be resumed.

The cooling of the rails in the above method may be accomplished in any suitable apparatus. In the apparatus illustrated in the accompanying drawing, the rails 10 are placed on and transversely of beams 11 which constitute the hotbed, and are moved progressively over the hotbed from one end to the other as indicated by the arrow in Fig. 1. While the rails are on the hotbed they are cooled by currents of air, set up by convection or otherwise, which rise upwardly between and about the rails. The rate of cooling is determined primarily or very largely by the rate of movement of these air currents. When the temperature of the surface of the rails drops to about 700° C. (1300° F.) or somewhat lower, they enter a closed chamber 12 having louvres 13 and 14 in its lower and upper walls to control and limit the upward passage of air about the rails in the chamber. Flaps 15 and 16 may be provided at the rail entrance and exit openings of the chamber.

The position or angle of the louvres 13 and 14 may be individually regulated to cool the rails to any rate, within limits, in the critical temperature range and immediately subsequent to it. The rails then pass under the flap 16 to the outer atmosphere, whereupon the usual more rapid cooling takes place. The rate of cooling of the rails after the retarded cooling in the chamber 12 has been completed may even be increased to compensate for the relatively longer time and greater space required for the period of retarded cooling.

It will be understood, however, that other apparatus may be used in the carrying on of the method of cooling in my invention and that various modifications of the form of the apparatus may be made. One such modification is to carry out the retarded and controlled cooling in a vertical, enclosed part of the hotbed, so arranged

that the rails in a horizontal position move up one side and down on the other, being discharged for final cooling on a hotbed of the ordinary type; in this case again, the flow of air past the cooling rails is controlled by suitable louvres or flaps.

5

What I claim is:

1. The method of treating rails which comprises heating the rail to temperatures above the critical temperature of the steel comprising the rail, cooling the rail to a temperature approximating the transformation temperature of the steel comprising the rail, equalizing the temperature differentials in said rail at said temperature and thereafter slowly and uniformly cooling the rail during the period of transformation and at least to temperatures approximating 550° C.

2. The method of treating rails which comprises heating the rail to temperatures above the critical temperature of the steel comprising the rail, cooling the rail to temperatures below the critical temperature but above about the transformation temperature of the steel comprising the rail, equalizing the temperature differentials in said rail resulting from said cooling and thereafter slowly and uniformly cooling the rail through the transformation temperature and to temperatures at least approximating 550° C.

3. The method of treating rails which comprises heating the rail to temperatures above the critical temperature of the steel comprising the rail, cooling the rail to temperatures approximating 700° C. but not below the transformation temperature of the said steel, equalizing the temperature differentials in said rail, slowly and uniformly cooling the rail through the said transformation temperature and at least to temperatures approximating 550° C. and thereafter cooling in any convenient manner to normal temperatures.

4. The method of manufacturing rails which comprises hot working the rail to the desired final size, cooling the rail to temperatures approximating the transformation temperature of the steel comprising the rail, equalizing the temperature differentials in said rail slowly and uniformly cooling the rail through said transformation temperature and to temperatures approximating 550° C. and thereafter cooling the rail in any convenient manner to normal temperatures.

5. The method of manufacturing rails which comprises hot working the rail to the desired final size, cooling the rail to a temperature below the critical temperature of the steel comprising the rail but above about the temperature of transformation, equalizing the temperature differentials in said rail, and slowly and uniformly cooling the rail through the said transformation temperature and to temperatures approximating 550° C. and thereafter cooling in any convenient manner to normal temperatures.

6. The method of manufacturing rails which comprises hot working the rail to the desired final size, cooling the rail to temperatures approximating 700° C. but above the transformation temperature of the steel comprising the rail, equalizing the temperature differentials in the rail, slowly and uniformly cooling the rail to temperatures approximating 550° C. and thereafter cooling in any convenient manner to normal temperatures.

7. In the manufacture of steel rails, the method of cooling the hot rolled rails which comprises rapidly cooling the rail to temperatures approximating the transformation temperature for the steel composition comprising the rail, re-

tarding the rate of cooling of the rail during the period of transformation to obtain a substantially uniform temperature throughout the heads of said rails and thereafter slowly and uniformly cooling said rails at least to temperatures approximating 550° C.

8. In the manufacture of steel rails, the method of cooling the hot rolled rails which comprises rapidly cooling the rail to temperatures approximating the transformation temperature for the steel composition comprising the rail, retarding the rate of cooling of the rail during the period of transformation to obtain a substantially uniform temperature throughout the heads of said rails, slowly and uniformly cooling said rails at least to temperatures approximating 550° C.

9. In the manufacture of steel rails, the method of cooling the hot rolled rails which comprises cooling the rail at any desired rate to a temperature below the critical temperature but above about the temperature of transformation of the steel comprising the said rail, equalizing the temperature differentials in the rail, slowly and uniformly cooling the rail through said transformation temperature at a rate substantially adapted to maintain all parts of the rail during transformation at substantially the same temperature, slowly and uniformly cooling the rail to temperatures approximating 550° C. and thereafter cooling the rail at a more rapid rate to atmospheric temperatures.

JOHN JOHNSTON. 15